

# UNITED STATES PATENT OFFICE.

JAMES ASTON, OF PITTSBURGH, PENNSYLVANIA, ASSIGNOR TO A. M. BYERS COMPANY,  
OF PITTSBURGH, PENNSYLVANIA.

## MANUFACTURE OF WROUGHT-IRON.

REISSUED

1,255,499.

Specification of Letters Patent.

Patented Feb. 5, 1918.

No Drawing.

Application filed August 18, 1917. Serial No. 186,830.

*To all whom it may concern:*

Be it known that I, JAMES ASTON, of Pittsburgh, in the county of Allegheny and State of Pennsylvania, have invented a new 5 and useful Improvement in the Manufacture of Wrought-Iron, of which the following is a full, clear, and exact description.

Heretofore the usual method employed in the manufacture of wrought-iron has been 10 the puddling process, which consists in refining pig-iron in a puddling or reverberatory furnace to remove the carbon, sulfur, and phosphorus from the iron, and then when the molten metal begins to lose its fluid- 15 ity or comes to nature in the form of a pasty mass, to work this mass in its bath of slag, whereby the slag remains incorporated with the iron, and a ball is formed which is re- 20 moved from the furnace and taken to a squeezer, and thence to rolls, producing blooms, billets, or muck bars of wrought-iron. The chief objections to this process are that skilled labor is required, the opera- 25 tion is slow and tedious, and only a small quantity of wrought-iron can be produced at each heat. The purpose of my invention therefore is to dispense with the skilled labor required in the puddling process, and to lessen the time ordinarily required in the 30 production of wrought-iron; and it consists in mechanically mixing disintegrated iron with a silicate or other suitable slag, raising the iron and slag to a welding heat, and then 35 squeezing and rolling the same into billets and bars. This may be accomplished by placing fagots or bundles of thin iron rods, or shavings and chips of iron, in a bath of molten iron silicate slag in a suitable fur- 40 nace, and allowing the iron to remain in the molten slag until it has attained a welding heat, and then removing the fagot or bundle of iron with the adhering slag and squeezing 45 and rolling the same in the manner commonly employed with puddled balls in the puddling process.

I will now describe my invention more fully, that others skilled in the art to which it appertains may employ the same.

Highly refined iron, produced by the Bes- 50 semer or open hearth process, is disinte-

grated by any suitable milling operation that produces chips or shavings, and these chips or shavings are formed into a bundle and placed in a molten bath of silicate slag in an open hearth or other suitable furnace, 55 where the iron is allowed to remain until it has attained a welding heat. The bundle of iron with the adhering slag is then removed from the furnace and taken to the squeezer where it is formed into blooms in 60 the usual manner. Instead of forming the chips and shavings into bundles, they may be placed in the slag loosely, and after the iron has come to a welding heat it can be formed into a ball in the slag by means of a clam 65 shovel or other suitable tool. Or, instead of chips and shavings of iron, fagots may be formed of iron rods into the interstices of which the slag will flow. Or, under certain conditions, the cold slag and the disinte- 70 grated iron may be placed on the hearth of the furnace together, as the heat required to bring the slag to a molten state will at the same time bring the iron to a welding heat or other forms of disintegrated iron may be 75 employed. Although I have described heating the iron in the bath of molten slag, I do not desire to limit myself thereto as the iron may be brought to a welding heat before it is mingled with the slag. Nor do I desire to 80 limit myself to a silicate slag as in certain cases other forms of slag may be desirable.

The advantages of my invention are that the refining of the iron, which may be accomplished in large quantities by the Bessemer or open hearth processes, is separate 85 from the operation which incorporates the silicate with the iron; and larger quantities of iron may be treated by my process in an open hearth furnace at one heat than can be 90 puddled. The result of this is a great saving in time and labor.

Having thus described my invention, what I claim and desire to secure by Letters Patent is—

1. The method of producing wrought-iron consisting in ringing refined iron to a welding heat in a silicate bath, and then squeezing and rolling the mingled slag and iron.

95

100

2. The method of producing wrought iron consisting in heating disintegrated refined iron when mingled with slag to a welding heat and then squeezing and rolling the same.

3. The method of producing wrought iron consisting in mingling disintegrated iron and molten slag, the point of fusion of which is lower than that of the iron, and then

squeezing and working the metal at a welding heat to a product.

In testimony whereof, I have hereunto set my hand.

JAMES ASTON.

Witnesses:

B. TROTTER,  
JAMES K. BAKEWELL.

Copies of this patent may be obtained for five cents each, by addressing the "Commissioner of Patents, Washington, D. C."